

April 3, 1951

H. L. SAUMS ET AL

2,547,047

METHOD OF PRODUCING INSULATED MAGNET WIRE

Filed May 22, 1947

3 Sheets-Sheet 1



April 3, 1951

H. L. SAUMS ET AL

2,547,047

METHOD OF PRODUCING INSULATED MAGNET WIRE

Filed May 22, 1947

3 Sheets-Sheet 2

**FIG. 3**



**FIG. 4**



INVENTORS  
HARRY L. SAUMS  
JOHN H. VAIL  
HOWARD W. STURGIS

BY  
*Dennis Edmonds, Morton and Parsons*  
ATTORNEYS

April 3, 1951

H. L. SAUMS ET AL

2,547,047

METHOD OF PRODUCING INSULATED MAGNET WIRE

Filed May 22, 1947

3 Sheets-Sheet 3



FIG. 6



FIG. 5

INVENTORS  
HARRY L. SAUMS  
JOHN H. VAIL  
HOWARD W. STURGIS

BY  
*Dennis, Edmonds, Morton and Garrows*  
ATTORNEYS

## UNITED STATES PATENT OFFICE

2,547,047

METHOD OF PRODUCING INSULATED  
MAGNET WIRE

Harry L. Saums, John H. Vail, and Howard W. Sturgis, Muskegon, Mich., assignors to Anaconda Wire and Cable Company, a corporation of Delaware

Application May 22, 1947, Serial No. 749,804

4 Claims. (Cl. 117—66)

1

This invention relates to insulated wire, particularly wire of the character known to the trade as magnet wire. The invention provides an improved method for producing such insulated wire, and novel apparatus in which the method of the invention may be carried out. Wire produced in accordance with the invention is a new product possessing improved characteristics, and the wire is itself therefore included within the scope of the invention.

A common type of magnet wire consists of a metallic wire having an insulating enamel coating. Methods heretofore known for producing such wires involve applying to the wire a number of coats of oleo-resin enamel, or some similar enamel, and baking the wire after applying each coat to dry and harden the enamel on the wire. The baking step has always been necessary in the commercial production of enameled magnet wires, because the only enamels heretofore successfully employed have been of the type requiring evaporation of solvent, with or without oxidation of the vehicle, to dry and harden the enamel film on the wire. The film produced by only one coat of these baked enamels is so thin as to be inadequate for electrical insulating purposes, and accordingly it has been commercial practice to apply a minimum of three coats and sometimes as many as twelve coats, with a baking step intermediate the application of each coat. The need for applying a number of coats of enamel has the effect, of course, of diminishing the amount of finished wire that can be produced per unit of time with a given amount of wire-enameling equipment.

Production of enameled wire by heretofore known methods is a slow process for still another reason. The drying and hardening of each coat of enamel requires baking for an appreciable length of time. There is a practical limit to the size of enameling ovens that can be built and operated economically, and even in ovens of the largest size deemed practical the rate at which the wire can be passed therethrough, and still allow adequate time for baking the enamel coat, is low—varying say from about 10 feet per minute for No. 10 A. W. G. (American Wire Gauge) wire to about 55 feet per minute for No. 39 A. W. G.

In order to obtain maximum production from an enameling oven, it must be operated at the highest temperature consistent with the maximum temperature the enamel can withstand without deterioration (in order to permit passage of the wires through the oven at the greatest

2

possible speed), and the wires must be closely spaced in the oven. Thus, enameling ovens are generally operated at a temperature of about 300° to 360° C., and the wire spacing is about 5 one-half inch. If the enameled wire is allowed to remain in the oven under these conditions for a period of time only slightly exceeding the normal baking time, due either to a variation in wire speed or to a break in the wire, the resulting overbaking will cause such deterioration of the enamel coating as to make the wire valueless. A high degree of skill is required of the operators of such ovens to avoid any such damage to the wire and to insure the production of 10 long lengths of uniformly baked enameled wire suitable for use in the electrical trade.

We have discovered that insulated magnet wire of excellent quality can be produced by passing a wire through a gelable lacquer maintained at 20 above its gelation temperature, and cooling the lacquer coated wire rapidly upon its withdrawal from the lacquer to a temperature below the gelation temperature of the lacquer. The resulting lacquer coated wire has been found to have excellent insulating qualities, adequate for many commercial uses, when only a single coat of such gelable lacquer is applied. The wire may be produced commercially in this manner without baking and at speeds even ten times or more faster than is possible by wire-enameling procedures 25 heretofore known. Uniformly coated wire may be thus produced without skilled attention, and the coating operation may be slowed or even completely stopped without deleteriously affecting the quality of the applied coating.

The gelable lacquers referred to herein are known to the chemical industry as such, or sometimes, as "gel lacquers" or "gelation lacquers." They are solutions of complex organic compounds, usually in the category of synthetic resins or plastics, which are fluid at moderately elevated temperatures (usually in the range of 120° to 200° F.) and solidify to a non-flowing self-supporting state by gelation upon cooling to a 40 temperature below 100° F. (usually near ordinary room temperature—about 70° F.). These gelable lacquers as such do not constitute a part of our present invention. Lacquers in which a cellulose ester is the solute constituent are being and have been developed. For example, United States patents to Fordyce et al. Nos. 2,319,051 through 2,319,055, describe gelable cellulose ester lacquers which are fluid at temperatures above 120° F. but form self-supporting non-flowing gels when the temperature is lowered to 45 50 55

below 100 F., and usually to about 70° F. or below. Our invention contemplates using such heretofore known lacquers, including those described in the above-noted patents and others as well, in the production of insulated magnet wire by our novel procedures and in our novel apparatus.

Gelable lacquers have heretofore been employed to produce organic films (as disclosed in the above-mentioned Fordyce et al. patents), and to produce quite heavy coatings by dipping methods on such articles as shoe heels, handles of kitchen utensils, tool handles, towel racks, steering wheels, and the like. Such articles are coated by dipping them in a hot gelable lacquer solution maintained at a temperature above the gelation temperature and by withdrawing the articles from the hot solution with a slow continuous motion no faster than the viscous excess lacquer can run back into the body of the hot solution. The rate of withdrawal is usually about one inch every six to twelve seconds, amounting to a linear speed of about 0.4 to about 0.8 foot per minute. This slow withdrawal rate is necessary because gelable lacquers in the liquid state are characterized by having a high viscosity, and an excessively thick and irregular accumulation of lacquer is formed on the article if it is withdrawn more rapidly. Upon cooling to a temperature below the critical gelation temperature, the lacquer sets in the form of a thick coating about 0.006 to about 0.030 inch in thickness. Although the thick lacquer coating may be gelled by cooling to a non-flowing state very quickly after removal of the article from the hot lacquer solution, the coated article must be allowed to dry for ten to twenty minutes or longer before the coating is sufficiently hard to withstand moderate handling; and in order for the coating to be hard enough to withstand the handling incident to normal use, it must be allowed to dry for a much longer time (usually a matter of hours).

Although the characteristics of the dip-coating procedures heretofore known for coating articles with a gelable lacquer, and the characteristics of the coatings so produced, have indicated that such procedures could not be used in the insulation of magnet wire (which must be withdrawn from the coating bath at a linear speed far in excess of that used in dip coating articles, and which must be handled by mechanical supports within an extremely short time interval after the wire is withdrawn from the coating solution), we have found it possible nonetheless to use such gelable lacquers to produce wholly satisfactory insulated wire.

We have found that when magnet wire is provided with such a coating of a gelable lacquer having a thickness less than 0.005 inch, and advantageously about 0.0001 to about 0.002 inch, the applied hot lacquer coating may be cooled to its gelation temperature and substantially complete evaporation of the lacquer solvent may be effected during passage of the wire at a relatively high speed from the coating bath to the first wire-supporting element positioned a reasonable distance from the bath. Contact of the coated wire with a supporting element such as a pulley wheel or sheave may be made safely without damaging the coating in about 1.5 minutes or less, and down to 0.075 minutes when fine wires are being coated, after application of the coating. By the end of this period the lacquer has gelled and the solvent has evaporated to such an extent as to permit such handling of the wire. The coated wire may

be wound upon a spool or in the form of an electrical coil within about 0.15 to 3 minutes after the wire passes through the coating solution, the actual time depending more or less on the size of the wire.

In any practical wire-coating operation, the linear speed of the wire implicit in the time figures given above is such that the coating thickness specified (less than 0.005 inch) is much less than can be obtained simply by drainage of the lacquer at its natural flow rate from the moving wire as it emerges from the lacquer bath.

Based on the foregoing findings, the method of our invention involves passing a wire beneath the surface of a body of gelable lacquer maintained at above its gelation temperature, limiting the thickness of the lacquer film remaining on the wire upon its withdrawal from the body of lacquer to less than that obtainable by the natural flow rate of the lacquer, and cooling the lacquer film on the wire to below its gelation temperature promptly upon withdrawal of the wire from the body of lacquer. It is generally advantageous, and in many cases possible, to regulate the thickness of the lacquer film so that normal magnet wire insulation is provided in a single pass of the wire through the body of lacquer. The rate at which the wire is passed through the body of lacquer is, in accordance with the invention, enormously greater than the rate at which gelable lacquers may be applied as dip coatings by the procedures heretofore known, and may even exceed by a substantial margin the rate at which magnet wires can be enameled by wire-enameling methods known heretofore. It is also possible to coil wire coated in accordance with the invention much sooner after application of the coating than has been possible in the production of magnet wires by heretofore known enameling methods.

Apparatus for producing magnet wire in accordance with the invention comprises basically a lacquer vessel, means for heating a body of gelation lacquer in said vessel to above its gelation temperature, a cooling zone maintained at a temperature below the gelation temperature of the lacquer, and means for continuously passing a wire to be insulated first through the body of lacquer and therefrom through the cooling zone. The same vessel which contains the lacquer advantageously also defines the cooling zone. In such an arrangement, the body of lacquer is in the lower portion of the vessel, and is heated therein to above its gelation temperature by heating coils or otherwise. In the upper portion of such vessel, above the surface of the lacquer, cooling coils or other cooling means are provided to maintain the temperature of the atmosphere below the gelation temperature.

The foregoing and other features of the invention are described below in some detail, with reference to the accompanying drawings, in which

Fig. 1 is a cross section through apparatus for producing wire in accordance with the invention;

Fig. 2 is a view on an enlarged scale of the grooved rotatable wheels shown in Fig. 1, taken substantially along the line 2-2 of Fig. 1;

Fig. 3 is a semi-logarithmic plot showing the linear speed at which wires of different sizes may be coated by enameling methods heretofore commercially employed compared with the method of the invention;

Fig. 4 is a semi-logarithmic plot of the time within which wires of different sizes, enameled by heretofore known commercial methods, may be

coiled after application of the enamel, compared with the time within which wires coated in accordance with the invention may be coiled;

Fig. 5 is a schematic cross section through a modified form of the apparatus shown in Fig. 1; and

Fig. 6 is a schematic cross section through another modified form of the apparatus shown in Fig. 1.

The apparatus shown in Figs. 1 and 2 comprises a vessel 10 containing a body of gelable lacquer solution 11. A spiral heating coil 12 immersed in the solution is provided to maintain the lacquer at above its gelation temperature. An inlet connection 13 and an outlet connection 14 are provided for admission and withdrawal of steam, hot oil or water, or other heating fluid. It is of course evident that various other heating means, such as a heating jacket surrounding the lower portion of the vessel 10, electrical heating windings inside or surrounding the lower portion of the vessel, or even a screen-enclosed flame impinging on the bottom of the vessel, or a hot plate on which the vessel rests, may serve as the heating means. The temperature at which the gelable lacquer is maintained by the heating means advantageously is thermostatically controlled.

The normal surface level 15 of the fluid gelation lacquer is well below the top of the vessel 10. Cooling coils 16 are arranged in the upper portion of the vessel 10 to cool the atmosphere in the cooling zone 17 (above the surface of the lacquer) to a temperature below the gelation temperature of the lacquer. This cooling zone not only serves to cool the lacquer coating on the wire to its gelation temperature, but also serves to condense the lacquer solvent vapor emanating from the body of heated lacquer solution, so as to assist (by gravity return to the solution of the condensed solvent vapor) in maintaining the composition of the solution. An inlet 18 and outlet 19 provide for the admission and withdrawal of cooling water or other cooling fluid to and from the cooling coils 16. As in the case of the heating coil 12, many other alternatives to the cooling coils 16 shown in the drawings may be provided for maintaining the temperature in the zone 17 at the proper value. In some cases, where room temperature is safely below the gelation temperature, no special provision for cooling need be made, other than to insure that the wire comes to the temperature of the room atmosphere.

A wire 20 to which a lacquer coating is to be applied is drawn from a spool 21 mounted at the side of the vessel 10. A freely rotatable idler wheel or roller 22 directs the wire 20 from the spool 21 downwardly into the vessel and into the lacquer solution 11. The wire passes around one of a pair of freely rotatable peripherally grooved wheels 23 and 24. These wheels are mounted so that they project a short distance into the body of lacquer 11, and the wire is coated with lacquer in the course of its passage therearound. The grooves in the wheel peripheries define an opening between their abutting faces through which the coated wire 25 emerges from the lacquer into the cooling zone 17.

From the cooling zone the coated wire passes around one or more wire-supporting pulleys 26 to a capstan 27. Conventional motive means are provided to rotate the capstan and draw the wire from the spool 21 continuously through the lacquer and thence through the cooling zone. The wire passes from the capstan to a traverse mechanism 28 which feeds it back and forth across

the face of a spool or other coil form 29 mounted on the spindle 30 of a suitably driven coiling head.

The arrangement of the peripherally grooved wheels 23 and 24 is shown on an enlarged scale in Fig. 2. Each of these wheels is freely rotatable on short axles 31 and 32, respectively. Collars 33 on the outer ends of the axles bear against the hubs 34 of the wheels and hold them in position. One of the wheels 23, preferably that around which the wire 20 passes, is mounted on an arm 35 depending from a bracket 36 and rigidly connected thereto. The other wheel 24 is mounted on a similar depending arm 37, but one which is pivotally mounted on the bracket 36 by a pivot pin 38. A tension spring 39 urges the pivoted arm 37 and the wheel 24 carried thereby toward the mating wheel 23, so that normally the peripheries of the two wheels abut.

Each of the wheels is formed with a peripheral groove 40, so that an opening 41 is defined at the abutting peripheries of the wheels. It is through this opening that the coated wire 25 emerges to pass into the cooling zone 17 of the vessel 10. Since the amount of lacquer that remains on the wire after its emergence from between the wheels depends on the size of the opening 41 in relation to the size of the wire, the grooves 40 should be of such size as to produce the desired thickness of the coating film.

Although V-shaped grooves 40 are shown in the drawings, the shape of the grooves is not critical. The advantage of V-shaped grooves is that a form tool for cutting such grooves to the correct depth is easily made. The grooves may, however, be semi-circular or rectangular in cross section, or of any other desired shape, provided only that they serve to define an opening of the proper size through which the wire can pass between the abutting peripheries of the wheels.

The peripherally grooved wheels 23 and 24, by their action in limiting the amount of lacquer remaining on the wire upon its withdrawal from the lacquer solution, insure production of an even coating of desired thickness about the wire. The small amount of flow necessary for the lacquer passing through the rectangular opening 41 to form a film of even thickness about the periphery of the circular wire occurs quite readily in the short time interval before the lacquer coating gels. It is for this reason that the shape of the grooves in the wheels 23 and 24 is not particularly critical. Grooved wheels of the characterized described are capable of applying a uniform coating of the desired thickness regardless of the linear speed of the wire. The grooved wheels have been found to operate effectively with lacquer solutions at viscosities up to about 300 poises, the maximum encountered in practice, and are capable of applying a coating of the desired thickness independently of the normal flow rate of the viscous lacquer solution.

We have found that die plates having simply a hole therein through which the wire is drawn are not particularly satisfactory in coating wires with gelation lacquers. It is impossible in practice to keep the wire centered at all times in the opening of such die plates, and in consequence such plates generally remove more lacquer from one side of the wire than from the other. Unless the rate of production is unduly limited the lacquer gels before it has an opportunity to flow to the extent necessary to form an even coating of uniform thickness completely about the periphery of the wire.

The lacquer solution 11 which fills the lower

portion of the vessel 10 may be any gelable lacquer which is fluid at a moderately elevated temperature but which gels to a non-flowing self-supporting solid, without evaporation of the solvent, when the temperature thereof is sufficiently lowered. Many lacquers of this character are known, and the preparation of still others is within the skill of workers in this field. Among the lacquers that we have used with success are those in which the solute constituent is an ester of cellulose and at least one fatty acid of one to four carbon atoms. Either a single ester such as cellulose acetate, or a mixed ester such as cellulose acetate-butyrate or cellulose acetate-propionate, may be used. Such lacquers are prepared by dissolving the cellulose ester in a suitable solvent, or mixture of solvents, in the correct proportions, and heating to a temperature above the gelation temperature. Many suitable solvents for gelable cellulose ester lacquers are available. For example, gelable cellulose ester lacquers have been prepared using one or more of the following solvents: alkylene dichlorides (e. g. propylene or butylene chloride), aliphatic alcohols, particularly the lower aliphatic monohydric alcohols containing five carbon atoms or less (e.g. ethyl alcohol, isopropyl alcohol, etc.), toluene, benzene, xylene and ligroin.

While we have obtained particularly satisfactory results using cellulose ester lacquers of the character referred to above and as disclosed in the aforesaid Fordyce et al. and other patents relating to such lacquers, the invention is not limited to the use of cellulose ester gelation lacquers. Gelation lacquers in which the solute constituent is polyethylene (polymerized ethylene) have also been used successfully. Gelation lacquers incorporating still other resinous plastic compositions as the solute, such as polyvinyl chloride, copolymers of vinyl chloride and vinyl acetate, and ethyl cellulose (a polymer prepared by reaction of ethyl chloride and cellulose), may also be employed in accordance with the invention.

We have obtained excellent results using a gelable lacquer composition composed of about 18% cellulose acetatebutyrate, 16.4% isopropanol and 65.6% commercial xylol. This lacquer had a viscosity between 900 and 1000 centipoises at 122 F. and a gelation temperature of about 70° F. The lacquer was maintained at a temperature between 140° and 160° F. in the vessel 10, although the lacquer could be maintained at a higher temperature up to that at which bubbling occurs (usually about 200° F.). Excellent coated wires, meeting or exceeding the specifications established for commercial enameled magnet wires, have been obtained by passing bare metallic wire through this lacquer solution, in the apparatus described above, at speeds ranging from 75 to 160 feet per minute. Equally satisfactory results are obtained using a cellulose acetate gelable lacquer composed of about 17% cellulose acetate, about 58% propylene chloride, and about 25% isopropyl alcohol; and using a cellulose acetate-propionate lacquer composed of about 20% cellulose acetate-propionate, 24% isopropyl alcohol, and 56% toluene.

We have also coated magnet wires in accordance with the invention with a gelable lacquer solution composed of 20% to 23% of an ethyl cellulose obtained on the market as "standard 50-centipoise, medium ethoxy ethyl cellulose" dissolved in commercial xylol. This lacquer solution was maintained at a temperature of about

200° F. in the vessel 10 and had a gelation temperature of about 70° F. Similar ethyl cellulose gelable lacquers were used in which the solvent was modified by the addition of a low boiling range aliphatic hydrocarbon solvent having a boiling range of 230° to 230° F. We have also modified the physical characteristics of coatings produced by such lacquers, by incorporating in the lacquer solution agents such as the Paraplex resins (copolymers of sebacic acid, glycerol, and ricinoleic acid).

We have in addition produced very satisfactory coated magnet wires by the process of the invention using a gelable "polyethylene lacquer" comprising, as far as we have been able to ascertain, about 20% polyethylene solids in toluol as a solvent. The lacquer was applied to the wire at a temperature of about 180° to 190° F.

Plasticizers may be incorporated in the gelable lacquer solutions, but generally, for wire coating purposes, it is preferable to omit the plasticizer. Unplasticized cellulose ester films deposited on wires in accordance with the invention are usually harder and more abrasion resistant than plasticized films, and yet are adequately flexible for the uses to which magnet wires are ordinarily put.

Colored and opaque coatings of gel lacquers can be produced by adding to the lacquer solution an appropriate dye or pigment which is compatible therewith. The dye should be soluble in the lacquer solution, and many such dyes are known which do not deleteriously affect the desirable characteristics of the gelled lacquer film on the wire. Pigments and other solid materials such as finely divided aluminum oxide, titanium dioxide, silicon dioxide, iron oxide, and the like, may be used as the coloring or opaques agent. By appropriate choice of the pigment and the amount thereof used in the lacquer, it is possible to modify other characteristics of the coating besides its color or opacity. For example, a sufficient amount of a metal oxide pigment in the coating will generally increase its resistance to heat.

In carrying out the method of our invention in apparatus such as that shown in Figs. 1 and 2, the wire 20 is drawn continuously from the spool 21 around the grooved wheel 23, whereby it is immersed in the body of lacquer 11. As the result of such immersion, the hot liquid lacquer wets and adheres to the surface of the wire. The temperature of the lacquer is maintained by the heating coils at above the gelation temperature and high enough to establish the desired lacquer viscosity, but preferably not so high that bubbles form in the solution (ordinarily bubble formation begins about 200° F. or higher). The wire is drawn upwardly through the opening 41 defined by the grooves in the abutting peripheries of the freely rotatable wheels 23 and 24, rotation of which is caused by the movement of the wire.

The opening 41 limits the thickness of the film of lacquer remaining on the wire after it has passed therethrough to less than could be obtained by the natural flow rate of the lacquer with the wire traveling at any reasonable coating speed. As the coated wire emerges from the opening 41, the coating remains liquid for just about long enough to flow into and form a uniform coating about the wire, and it then solidifies by gelation to form a self-supporting film on the wire.

In coating wire with a gelable cellulose ace-

tate-butyrate lacquer maintained at a coating temperature of about 140° to 160° F., we have found that gelation and solvent evaporation take place satisfactorily in the cooling zone 17 without the aid of cooling by the cooling coils. The atmosphere at ordinary room temperature suffices to accomplish these results. However, improved gelation and, more particularly, improved solvent recovery by condensation of solvent vapor in the cooling zone 17, have been obtained by lowering the temperature of the cooling zone 17 to below room temperature by the use of cold tap water circulating through the cooling coils.

Whether or not the cooling coils are used to cool the zone 17 to below room temperature, gelation and solvent evaporation take place so rapidly that, with the wire moving at normal coating speeds, the coated wire can be touched lightly with the fingers without damage to the film at a point about 2 or 3 feet above the top of the vessel 10. Solvent evaporation continues as the coated wire 25 travels toward the supporting pulley 26, and by the time the wire reaches it gelation is complete and solvent evaporation has advanced to the point that the coated wire may be passed over the pulley without damage to the coating film. In general, for ordinary coating speeds, a distance of about 15 feet between the grooved wheels 23 and 24 and the upper pulley 26 is sufficient to permit quite complete hardening of the coating. This distance may of course be varied, if desired, depending upon the wire size and coating speed and thickness. For example, in coating fine wires such as No. 37 A. W. G., a distance somewhat less than 15 feet is usually sufficient, whereas with relatively coarse wires such as No. 15 A. W. G. a somewhat greater distance may be preferable, particularly if a thick coating of the lacquer is applied. By establishing a distance between the upper pulley 26 and the capstan 27 approximately equal to the distance between the upper pulley 26 and the grooved wheels 23 and 24, the coating film will be sufficiently hard to withstand the distortion caused by the capstan and by the coiling operation, which may follow immediately.

Wires of any size may be coated by the method and apparatus of the invention. In the case of the larger wires, such as No. 14 to No. 20 A. W. G., the rate of solvent evaporation from the gelled coating may be increased by gently heating the coating on the wire over a portion of the distance between the top of the vessel 10 and the upper pulley 26. Such heating may be accomplished by passing the wire through a steam coil, or by infra-red heating lamps, or in any other desired manner.

As pointed out above, the linear speed with which wires can be enameled in conventional enameling ovens depends on the size of the wire; and the same is more or less true in coating wires in accordance with the invention. The coating speeds involved in the method of the invention are indicated in Fig. 3 of the drawings, wherein coating speeds in feet per minute are plotted against the size (A. W. G.) of the wire being coated. The line *a*—*b* on Fig. 3 indicates substantially the maximum linear speed with which it has been possible heretofore to enamel wires in commercial practice with oleo-resin enamels requiring baking. An important commercial advantage of the new method is that it permits coating to proceed at a much higher linear rate of travel of the wire. The line *c*—*d*

of Fig. 3 indicates a fair average normal coating speed for coating wires of different sizes in accordance with the invention, although in particular cases a somewhat lower or substantially higher coating speed may be preferable; and the line *e*—*f* is indicative of speeds that actually have been attained in some cases. Ordinarily commercial wire coating in accordance with the invention will be conducted at speeds at least about double those attainable in baking-enamel coating operations. If the linear rate of withdrawal of articles being coated by the dip methods heretofore known for applying gelable lacquers were plotted to scale on Fig. 3, the speed of application of such thin coatings as are required for magnet wire insulation would lead to a curve that would be virtually indistinguishable from the Wire Size axis of the plot. It is evident from this plot that wires can be coated in accordance with the invention much more rapidly than with enamels that require baking (i. e., they can be coated at a rate in excess of the rate shown by the line *a*—*b* of Fig. 3), and enormously more rapidly than would be possible by heretofore known dip methods.

Related to the high coating speed attainable is the very short time that need elapse between applying the lacquer and coiling a wire coated in accordance with the invention. Coiling may be either on spools for convenience in handling, or in the form of finished electrical coils for the electrical industry. Fig. 4 is a plot, against wire size, of the time elapsed between application of the coating and coiling of the wire in the cases (1) of wires coated in accordance with the invention and (2) in accordance with heretofore known commercial methods. The line *g*—*h* of Fig. 4 indicates the minimum time within which wires of different sizes may be coiled commercially after coating with oleoresin enamels and baking. The elapsed time between immersing of any section of the wire in the lacquer and coiling of said section may, in accordance with the invention, be less than that indicated by the line *g*—*h*. The line *j*—*k* of Fig. 4 indicates a fair average time to allow in ordinary cases between application of lacquers in accordance with the invention and coiling of the coated wire. It is clear from this plot that wire coated in accordance with the invention may be coiled much sooner after application of the coating composition than is the case in the commercial wire-enameling procedures heretofore known. The short time interval between coating and coiling that is attainable in accordance with the invention may be contrasted with the time of several hours required for drying and hardening the thick gelable lacquer coatings formed by heretofore known dipping methods on tool handles and other such articles.

The line *m*—*n* plotted on Fig. 4 indicates the very short time interval that need elapse between application of the enamel and passage of the coated wire over the first supporting pulley or sheave after emergence of the wire from the body of lacquer. Within this period of time the lacquer may be gelled and sufficient solvent evaporated to produce a hard enough coating to withstand the forces to which it is subjected in being drawn over the support. In general the normal maximum elapsed time between the passage of any section of the wire through the lacquer and passage of the same section over the supporting sheave is less than about 1.5 minutes, and in the case of fine wires (say No. 40 A. W. G.)

it may be only 4.5 seconds (0.075 minute) or less.

As hereinbefore stated, wire prepared in accordance with the invention may be wound into finished electrical coils directly after coating, as a last step in a conjoint wire-coating and coil-winding operation. This represents the fulfillment of a desire that has long been felt in the magnet wire industry, but one that previously has not been attained because of the limitations imposed by the wire-enameling procedures heretofore commercially available. In winding electrical coils it is generally necessary from time to time to start and stop the movement of wire to the coil winder, and sometimes to vary the linear speed of wire travel. It is not feasible to interrupt the passage of wire through an enameling oven, or vary the speed with which it passes through the oven, for the reasons already given. Furthermore, it is not economically practical to limit coil winding to the speeds attainable in producing baked-enamel coated wires, or to subject it to the production hazards incident to breakage of the wire during the course of the coating operation. Our new wire coating method is not subject to these limitations. The coating speeds attainable are commensurate with commercial coil winding speeds, and passage of the wire through the body of gelable lacquer may be slowed down or speeded up, or even stopped altogether, as the occasion to do so arises, without deleteriously affecting the thickness or quality of the coating on the wire. Whereas an interruption in the passage of wire through a commercial wire enameling oven almost invariably results in ruining the wire, an interruption in the new coating operation has no significant effect on the wire, and the passage of the wire through the gelable lacquer may be resumed after an interruption without discarding any portion of the wire.

Various modifications may be made in the method and apparatus described above. For example, in producing wires with fairly thick coatings, it may be desirable to modify the apparatus as shown in Fig. 5. This modification involves providing an idler pulley or sheave 42 below the first pulley 26 over which the wire passes after emerging from the lacquer, and a second idler 43 about at the elevation of the first pulley 26. The coated wire passes upwardly around the first pulley 26, downwardly and around the idler 42, and thence upwardly and around the second idler 43 to the capstan 27. The extra wire path length provided in this modification between the coating bath and the capstan allows, at a given wire speed, some additional time for solvent evaporation, in those cases where such is desirable.

It is ordinarily possible and desirable to apply a coating of adequate thickness to provide normal magnet wire insulation in a single pass of initially bare wire through the body of gelable lacquer. Coating thicknesses between 0.0001 inch and 0.002 inch are quite easily produced in accordance with the invention in a single pass through the lacquer, and thicknesses in this range (commonly near 0.0005 inch) are those usually desired for magnet wire insulation. Hence a feature of the invention is that in many cases the wire may be packaged for the electrical trade (either as a spool or coil of wire for convenient handling, or as a finished electrical or magnet coil) after but a single pass through the gelable lacquer coating solution.

For some purposes magnet wires having coat-

ings up to 0.005 inch are desirable, and for producing such wires apparatus modified as shown in Fig. 6 may be used with advantage. In this modification a second set of coating rollers 44 and 45, similar to the first set of rollers 23 and 24 described above, is mounted in the vessel 10 at the gelable lacquer surface. A second supporting pulley or sheave 46 similar to the first such pulley 26 also is provided. The incoming wire 20 passes down and through the body of gelable lacquer, around one of the rollers 24, and up to and around the supporting pulley 26. Thence the wire passes again into the body of lacquer and around a roller 44 of the second set to the second supporting pulley 46, from which it passes to the capstan 27. Thus two coats of the lacquer are applied to the wire in a single operation. We have found that a considerable number of coats may be applied thus directly after gelation of the previous coat, without injuring the coat or coats previously applied. There is no advantage, so far as insulating magnet wires are concerned, however, in applying more than two coats. We have been able to develop coating thicknesses up to 0.016 inch in only two passes of the wire through the lacquer, and so two coats may be regarded as the maximum necessary for ordinary wire coating operations even in those cases where thicker-than-usual coatings are desired.

Magnet wire produced in accordance with the invention is the equal of conventional enameled magnet wire in many respects, and it is superior in some respects. For example, magnet wire comprising a metallic conductor having thereon a thin, substantially continuous insulating film of an ester of cellulose and one or more fatty acids containing one to four carbon atoms (e. g. cellulose acetate-butyrate) applied directly in contact with the conductor surface, easily passes the quality acceptance tests established for ordinary enameled wire. The cellulose ester coating possesses high abrasion resistance. It is substantially insoluble in and not appreciably softened by petroleum oils, water or other liquids to which it is likely to be exposed in service. The wire may be bent on a mandrel of its own diameter without cracking the coating, even when the coating is unplasticized. The insulation resistance is high, even after prolonged exposure at a temperature of 120° F. to an atmosphere saturated with water vapor. The dielectric strength is likewise high. Continuity of the film is substantially equal to that of ordinary enameled wire. The "Q" value of coils wound from the new wire generally is substantially higher than that of coils wound from ordinary enameled wires. (The "Q" value of an electrical coil indicates the magnitude of the ratio of the amount of energy stored in the coil to the amount of energy dissipated therein for cycle of an alternating current flowing therethrough. A high "Q" value, which indicates that the coil will dissipate only a small amount of the power supplied to it or passed through it, is much desired in magnet wire coils employed in radio circuits and other fairly high frequency alternating current devices.)

Another feature of wires coated with a gelable lacquer in accordance with the invention is the ease with which the coating may be removed from the wire for making electrical connections. For example, the insulation may be removed readily from wires coated with a cellulose acetate-butyrate gel lacquer by dipping the wire in acetone. This leaves a clean wire sur-

face to which electrical connections may easily be made by soldering or otherwise. This is an outstanding advantage of the gel lacquer coated wire over baked enamel coated wire from which the enamel can be removed only by scraping or by the use of an abrasive such as sandpaper, or by powerful solvents. Sandpapering is slow and frequently causes breakage of fine wires, and the solvents which will remove heretofore known baked enamels are expensive, toxic, must be handled carefully and must be thoroughly washed from the wire.

Coatings applied to wires in accordance with the invention do not adhere to the wire as do baked enamel coatings, but this is not a disadvantage, and is even an advantage in that it permits easy mechanical stripping of the coating if a suitable solvent is not at hand. Solvent evaporation that ensues after gelation of the coating is accompanied by shrinkage of the coating tightly about the wire, so that there is no danger of the coating slipping on the wire accidentally.

It is evident from the foregoing that the invention provides a magnet wire possessing in a large measure the properties desired in such wires, and yet that can be made by the method and with the apparatus of the invention much more rapidly and with much less costly equipment than heretofore known enameled wires.

We claim:

1. The method of producing insulated magnet wire which comprises passing a wire through a body of gelable lacquer which is maintained at substantially atmospheric pressure and which is maintained in the liquid state by being heated to above its gelation temperature, withdrawing the wire from the body of lacquer and substantially simultaneously limiting the thickness of the lacquer film on the wire to less than 0.005 inch and less than that obtainable by the natural flow rate of the lacquer by passing the wire through a restricted opening formed by two arcuate members, at least one of which rotates in a direction such that its edge adjacent the wire moves in the same direction as the movement of the wire through the opening, and cooling the lacquer film on the wire to below its gelation temperature promptly upon withdrawal of the wire from the restricted opening.

2. The method of producing insulated magnet wire which comprises passing a wire through a body of gelable lacquer which is maintained at substantially atmospheric pressure and which is maintained in the liquid state by being heated to above its gelation temperature, withdrawing the wire from the body of lacquer and substantially simultaneously limiting the thickness of the lacquer film on the wire to less than 0.005 inch and less than that obtainable by the natural flow rate of the lacquer by passing the wire through a restricted opening formed by two arcuate members, at least one of which rotates in a direction such that its edge adjacent the wire moves in the same direction as the movement of the wire through the opening, and cooling the lacquer film on the wire to below its gelation temperature promptly upon withdrawal of the wire from the restricted opening, the rate of passage of the wire through the body of lacquer and through the restricted opening in relation to the size of the wire being at least about equal to the rate shown by the line *c-d* of Fig. 3 of the accompanying drawings.

3. The continuous method of producing an electric coil which comprises passing a metallic wire through a body of gelable lacquer which is maintained at substantially atmospheric pressure and which is maintained in the liquid state by being heated to above its gelation temperature, withdrawing the wire from the body of lacquer and substantially simultaneously limiting the thickness of the lacquer film remaining on the wire to less than 0.005 inch and less than that obtainable by the natural flow rate of the lacquer by passing the wire through a restricted opening formed by two arcuate members at least one of which rotates in a direction such that its edge adjacent the wire moves in the same direction as the movement of the wire through the opening, cooling the lacquer film on the wire to below its gelation temperature promptly upon withdrawal of the wire from the restricted opening, and winding the wire into an electric coil of desired size and shape directly after gelation of the lacquer coating and as the final step in a conjoint wire-coating and coil-winding operation.

4. The continuous method of producing a coil of insulated wire which comprises passing a metallic wire through a body of gelable lacquer which is maintained at substantially atmospheric pressure and which is maintained in the liquid state by being heated to above its gelation temperature, withdrawing the wire from the body of lacquer and substantially simultaneously limiting the thickness of the lacquer film remaining on the wire to less than 0.005 inch and less than that obtainable by the natural flow rate of the lacquer by passing the wire through a restricted opening formed by two arcuate members at least one of which rotates in a direction such that its edge adjacent the wire moves in the same direction as the movement of the wire through the opening, cooling the lacquer film on the wire to below its gelation temperature promptly upon withdrawal of the wire from the restricted opening, and winding the wire into a coil of desired size and shape directly after gelation of the lacquer coating and as the final step in a conjoint wire-coating and coiling operation, the elapsed time between immersion of any section of the wire in the body of lacquer and coiling of said section, in relation to the size of the wire, being not appreciably greater than the time shown by the line *j-k* of Fig. 4 of the accompanying drawings.

HARRY L. SAUMS.  
JOHN H. VAIL.  
HOWARD W. STURGIS.

#### REFERENCES CITED

The following references are of record in the file of this patent:

#### UNITED STATES PATENTS

| Number    | Name        | Date          |
|-----------|-------------|---------------|
| 862,935   | Pfanstiehl  | Aug. 13, 1907 |
| 1,531,259 | Turner      | Mar. 24, 1925 |
| 1,993,838 | Hagedorn    | Mar. 12, 1935 |
| 2,044,970 | Candy       | June 23, 1936 |
| 2,051,944 | Hershberger | Aug. 25, 1936 |
| 2,156,607 | Schon       | May 2, 1939   |
| 2,197,622 | Sendzimir   | Apr. 16, 1940 |
| 2,291,670 | Wiley       | Aug. 4, 1942  |
| 2,308,638 | Balthis     | Jan. 19, 1943 |
| 2,315,645 | Newton      | Apr. 6, 1943  |
| 2,350,742 | Fordyce     | June 6, 1944  |